

*Saml. Wetherill Imp<sup>t<sub>3</sub></sup> in Appa. for Manufacture  
of White Oxide of Zinc.*



*Witnesses.*  
H. Scott  
A. DeLacy.

*Inventor:*  
Saml. Wetherill  
by atty  
L. M. Sibley

# United States Patent Office.

SAMUEL WETHERILL, OF PHILADELPHIA, PENNSYLVANIA.

Letters Patent No. 73,146, dated January 7, 1868.

## IMPROVED PROCESS OF MANUFACTURING WHITE OXIDE OF ZINC.

The Schedule referred to in these Letters Patent and making part of the same.

TO ALL WHOM IT MAY CONCERN:

Be it known that I, SAMUEL WETHERILL, of Philadelphia, of Philadelphia county, in the State of Pennsylvania, have invented certain new and useful Improvements in Process for the Manufacture of White Oxide of Zinc; and I do hereby declare that the following is a full and exact description thereof, reference being had to the accompanying drawings, making part of this application.

Previous to my present invention, the manufacture of white oxide of zinc, in the United States, has been carried on by the process described in Letters Patent granted to me in 1855, which is adapted to the reduction of the zinc ores with anthracite coal, and the two or three establishments working under (or upon the process described in) my said patent have about supplied the entire demand; but the increased expenses of deep mining, and the tendency of calamine deposits to run into sulphurets, and the scarcity of rich ores, have induced to a much greater cost of production than was sustained some time ago.

Notwithstanding the lavish expenditures of money, no new deposits of zinc ores have been discovered within reach of anthracite coal; and the enormous deposits of carbonate of zinc in Virginia, (S. W.) East Tennessee, Northern Arkansas, Missouri, Iowa, Illinois, and Wisconsin, together with the large deposits of bituminous coal in the Richmond basin, Tennessee, Great Illinois, and West Mississippi coal-fields, will come into competition now, and may supply the demand for a cheap oxide. But it will be found practically impossible, in the employment of these supplies, to coke large quantities of this bituminous coal, or convert into charcoal large quantities of wood, to carry on the process of manufacturing white oxide, and at the same time have either of these last-named substances free from coal-black, *i. e.*, lamp-black is specifically nearly as light as the flakes of white oxide, and particles of it will travel with the white oxide through all the known processes of separation, and will soil the products. It is apparent that some plan of avoiding this difficulty will be a great desideratum, and that by overcoming this difficulty, arising in the use, under the known processes, of the bituminous coal, or wood, a cheap article may be supplied to the market.

To accomplish these desirable ends is the main object of my present invention, which consists in causing the vapors of combustion, from coal, charcoal, or wood, (in the manufacture of white oxide,) to pass through incandescent carbon, whereby the coal-black and oxygen are consumed, and the oxide of zinc vapor is reduced to the condition of a metallic vapor of zinc, and furnishing such metallic vapor with the necessary supply of oxygen by means of a hot blast, igniting and consuming any specula of coal-black which might pass through the incandescent coal, all as hereinafter more fully described.

To enable those skilled in the art to which my invention relates to more fully understand it, I will proceed to describe more fully my improved method or process of manufacturing white oxide of zinc, referring by letters to the accompanying drawings, in which I have illustrated an apparatus for carrying out my said invention.

Figure 1 is a top view, and

Figure 2 is a front elevation of a furnace for conducting my new process, and which is similar to the furnace employed by me under my formerly patented process, but with the addition of two auxiliary furnaces and a hot blast, as will be presently explained.

Figure 3 is a vertical section at the line *x x*.

Figure 4 is a vertical section at the line *y y*, and

Figure 5 is a vertical section at the line *z z*.

In the several figures I have designated the same parts by the same letters of reference.

A is the main furnace-chamber, and B the grate-bars or perforated bed of the furnace. C is its ash-pit, and D the openings, through which the furnace is charged. E E are the cold-blast flues, and *e e* the passages leading from them to supply the cold blast to the furnace. This much of the apparatus or structure is about similar to that heretofore employed in carrying out the process or method of manufacture described in my previous patent. On each side of the furnace A is arranged a chamber, F F, beneath which is a conduit or passage, H H. These chambers, F F, are completely covered by the crown-arch A' of the furnace, and communicate with the chamber A only by means of ports or openings *d d*, and the bottoms of said chambers are formed of perforated refractory tile, *ff*, the apertures of which tile constitute numerous passages of communication between said chambers F F and the oxide-flues or passages H H, for purposes to be presently explained.

G G are the flues, through which the products of combustion are carried off to the separating and catching-apparatus, and g g are air-tubes, to which a supply of air is fed, and in which the air is heated, and from which the hot blast is supplied to the passages H H, as will be presently explained. The flues H H and chambers F F have doors i i and k k, through which access may be had to said flues and chambers when desired. a is the door of the ash-pit.

Having so far alluded in detail to the several parts of the apparatus employed, I will now explain the procedure of my new or improved process, as practised in the apparatus aliuded to.

A fire, of small coke, having been thoroughly ignited upon the perforated iron plate or grate B, of the centre or main furnace A, and the auxiliary furnaces or chambers F F having been supplied with beds of incandescent coals, of coke or charcoal, about up to the level of the lower sides of the ports d d d, the charge of ore and coke is put into the furnace A, through the charging-ponings D, which are stopped by a mass of the charging-materials. Of course the ore is previously crushed by any of the known means, and mixed with an equal bulk of wetted coke, or with a larger bulk of wetted charcoal, in the manner well known to those conversant with the art. When the furnace shall have been thus charged, the chambers F F filled with incandescent coals, and the fire thoroughly going, so that the zinc vapors arise, the hot blast is turned on to the oxide-flues H H, the hot blast being supplied from the tubes g g, which are so arranged, as shown, on the crown-arch of the furnace, that a supply of cold air, fed or forced into their upper ends, becomes heated before it escapes from their lower ends into the chambers H H.

The products of combustion having no other source of escape, are compelled to pass through the ports d d d, and thence down through the masses of incandescent coals, in chambers F F, and through the perforated tiles f f, into the oxide-flues H H, where they come into contact with and are carried off to the flues G G by the hot blast. And by being thus drawn through the incandescent carbon-chambers and hot-blast flues, the zinc vapor is reoxidized, and all the undecomposed specula of carbon which may have passed through the incandescent coals are consumed. After all the zinc shall have been expelled in the operation just explained, a damper may be closed, or inserted, at the termination of the oxide-flues, the old charge, if necessary, taken out, a fresh bed of small coke introduced and well ignited, and a new charge put in, and the operation repeated or continued, the incandescent chambers being always kept supplied with fresh coals. The product of my new process, as described, will be a beautiful white oxide, free from smut and coal-specula.

Although I have described my process as particularly applicable in the use of bituminous coal, and its greatest advantages result from its use with such kind of material as could not be otherwise successfully used in the manufacture of white oxide of zinc, nevertheless my invention, it will be understood, may be applied with considerable advantage to the manufacture of white oxide with anthracite coal; since in the present process of manufacture, undecomposed particles of coal are carried or "ballooned" along, by the force of the blast, past the tower and cooling-room, and soil the oxide, which objection will be overcome by my present invention.

A ravel or iron spatula may be employed to clean the perforated tiles f f of ashes, which, together with what oxide may collect in the flues H H, are removed from the latter, and may be mixed with the material of the charge for the furnace.

Having fully explained my new process, together with a suitable means of carrying the same into practice, so that one skilled in the art can fully comprehend it, what I claim as new, and desire to secure by Letters Patent, is—

Passing the products of combustion from the furnace into an auxiliary chamber or chambers, containing incandescent carbon, and thence through the incandescent coals, into contact with a hot blast, substantially as and for the purposes described.

In testimony whereof, I have hereunto set my hand and seal, this twenty-third day of October, 1867.

SAMUEL WETHERILL. [L. S.]

Witnesses:

W. C. WETHERILL,  
S. P. WETHERILL.